

## UNITED STATES PATENT OFFICE

2,308,853

## ARTICLE OF RESIN BONDED ABRASIVE GRAINS

Carl E. Barnes, Cambridge, Mass., assignor to  
Norton Company, Worcester, Mass., a corpora-  
tion of Massachusetts

No Drawing. Application August 25, 1941,  
Serial No. 408,195

10 Claims. (Cl. 51—298)

This invention relates to abrasive articles and more particularly to articles made of abrasive grains bonded by a resin formed of polymerized unsaturated methylene compounds.

Methyl methacrylate and similar polymerizable substances will serve as a bond for abrasive grains; but for various abrasive purposes, they have undesired characteristics, such as being not hard or strong enough or having too low a softening point or flowing too readily or smearing over the face of a grinding wheel when used in a dry grinding operation.

One object of my invention is to provide an improved abrasive article, such as a grinding wheel, which is made of abrasive grains bonded by polymerized unsaturated methylene compounds and which has a suitable hardness, strength, resistance to heat or other required physical characteristics.

Methyl methacrylate in its monomeric form contains the polymerizable unsaturated group  $\text{CH}_2=\text{C}-$ , and it is considered to polymerize by a rearrangement of the primary valence bonds in such a way as to form linear chains having the group  $\text{CH}_2-\text{C}-$  as a repeating unit. The linear chain type of ester may be interpolymerized with a further polymerizable compound containing two of the unsaturated  $\text{CH}_2=\text{C}-$  groups which are independently polymerizable. During polymerization the growing chains incorporate the  $\text{CH}_2$  groups of both substances and form an interpolymer having a three dimensional structure which is harder or has a higher resistance to heat or is less soluble or shows other different characteristics.

I have found that the vinyl and isopropenyl acrylates, chloracrylates and methacrylates, which have two of the unsaturated methylene groups, may be used to cross link various linear chain types of base substances, such as methyl methacrylate, to form interpolymers which serve as useful bonds for abrasive grains.

A further object of the invention is, therefore, to provide abrasive articles which comprise such interpolymerized substances and to form a series of abrasive bodies of widely different characteristics which will serve many useful purposes. Further objects will be apparent in the following disclosure.

In accordance with this invention, I propose to make various types of abrasive articles, such as grinding wheels, sharpening stones, cutting-off wheels and honing, lapping and polishing devices, by bonding abrasive grains, such as crystalline alumina, silicon carbide, boron carbide,

diamonds and other types of abrasive material, with resin substances formed of copolymers of the esters of acrylic acid, chloracrylic acid or methacrylic acid and the lower aliphatic alcohols having not over four carbon atoms, or mixtures of said esters, which are copolymerized with a suitable amount of a vinyl or propenyl acrylate or chloracrylate or methacrylate or mixtures thereof, and with or without other modifying substances. The hardness, strength, adhesion, resistance to heat, softening point and other physical characteristics of the bond are determined by the nature and the proportions of the bond ingredients and the method employed for making the article. By varying the amount of the cross linking agent, the strength and other physical characteristics of the bond may vary from approximately those of the linear chain ester to those of the cross linking agent.

15 The grinding wheel structure, as determined by the volume percentages of the abrasive grains, bond and pores, is governed in part by the relative proportions of the bond and grains used.

20 The grinding wheel structure, as determined by the volume percentages of the abrasive grains, bond and pores, is governed in part by the relative proportions of the bond and grains used.

The base substance of the bond is made up primarily of an ester of methyl, ethyl, propyl or butyl alcohol and acrylic acid, chloracrylic acid or methacrylic acid. The properties of these various substances are exemplified in the following table:

Polymers of methacrylic acid esters

|                                                         | Methyl | Ethyl | n-<br>Propyl | n-<br>Butyl | Iso-<br>butyl |
|---------------------------------------------------------|--------|-------|--------------|-------------|---------------|
| 35 Hardness (Pfund), G at<br>25° C.                     | 220    | 141   | 100          | 1           | 210           |
| Tensile strength, lbs./sq.<br>in.                       | 9000   | 5000  | 4000         | 1000        | 3400          |
| Impact strength (Dyn-<br>stat), kg.cm./cm. <sup>2</sup> | 10.5   | 7.1   | 6.5          | 11.5        | 1.6           |

40 It has also been found that comparatively hard resins are formed of the methacrylic acid esters of those alcohols which are branched as much as possible, i. e., the methyl, ethyl, iso-propyl and tertiary butyl alcohol esters of methacrylic acid; while much softer resins are formed of the remaining esters of less than a maximum branching, i. e. those of the normal propyl, normal primary butyl, normal secondary butyl and primary isobutyl alcohols. In general, the hardness and the thermal yield point decrease with the increase in molecular weight of the esterified alcohol. For example, methyl methacrylate softens above 100° C. while n-butyl methacrylate is soft and flexible at room tem-

45

50

55

perature. However, the branching of the alcohol materially affects these various properties, as shown by the fact that isopropyl alcohol forms a methacrylate resin that is almost as hard as is polymerized methyl methacrylate. Also, the isobutyl ester is much harder and has a higher softening point and is less flexible than the straight chain butyl ester. The tensile strength of the straight chain ester falls off as the molecular weight of the alcohol increases. Hence, these various esters have widely varying properties.

When any of these base substances are copolymerized with the vinyl or isopropenyl acrylates, chloracrylates or methacrylates, it is found that the interpolymers have similarly variable characteristics depending upon the nature and the proportions of the ingredients selected. Hence, by suitably choosing a linear chain type of ester as a base substance and modifying it with a suitable vinyl or isopropenyl ester, I may make abrasive bonds of widely different properties.

The linear chain types of esters may be obtained from suitable commercial sources or manufactured in accordance with standard procedure. The vinyl or isopropenyl compounds may be made by methods exemplified by the production of vinyl methacrylate, which may be prepared by the addition of acetylene to methacrylic acid in the presence of a mercuric sulfate catalyst. One suitable procedure is as follows:

Five grams of mercuric oxide are dissolved in one hundred cubic centimeters of glacial acetic acid heated to a temperature of eighty-five to ninety degrees centigrade with vigorous stirring. To this mixture is added three and three tenths cubic centimeters (one per cent excess) of concentrated sulfuric acid mixed with five cubic centimeters of glacial acetic acid, and this mixture is added dropwise with stirring to the mercuric acetate solution. The mercuric sulfate is then allowed to settle and the greater part of the acetic acid drawn off by suction. Most of the sulfuric acid is washed out of the catalyst by the addition of one hundred cubic centimeters of glacial acetic acid and drawing off all but about twenty-five cubic centimeters.

To this catalyst, one hundred cubic centimeters of one hundred per cent methacrylic acid containing pyrogallol as a polymerization inhibitor is added, and the mixture is heated to 85 to 90° C. Acetylene gas, after passing through sulfuric acid, is added to the mixture at the rate of about eight liters per hour. The gases issuing from the reaction flask are passed through a trap cooled in ice water which collects a considerable quantity of vinyl methacrylate. At the end of six or eight hours, the catalyst is filtered off and the filtrate is combined with the liquid from the trap, the mixture diluted with ether and the ether solution washed with aqueous sodium carbonate until neutral. After drying the ether solution with calcium chloride, it is distilled. Ether and vinyl acetate distill off and are not condensed. The first product collected is vinyl methacrylate which boils at forty-eight degrees at sixty millimeters. The next product collected is ethyldene dimethacrylate which boils at 89 to 91° C. at eleven millimeters pressure. Conditions may be changed to give a greater yield of vinyl methacrylate by increasing the rate of flow of acetylene and condensing the vinyl methacrylate in the trap outside the reaction mixture, thereby hindering the secondary reaction

which gives ethyldene dimethacrylate. Vinyl methacrylate rapidly polymerizes at room temperature to form a hard, transparent, colorless resin having an index of refraction of 1.503. This polymer is insoluble and infusible.

By employing propyne or methyl-acetylene  $\text{CH}_3\text{C}\equiv\text{CH}$  in place of acetylene, I may make isopropenyl methacrylate. The other homologues may be similarly prepared by using acrylic acid or chloracrylic acid instead of methacrylic acid in the above defined procedure.

I may alternately prepare vinyl methacrylate as follows:

(a) By the addition of methacryl chloride to acetaldehyde and subsequently dehydrohalogenating the product.

(b) By esterifying ethylene chlorhydrin with methacryl chloride and dehydrohalogenating the chloroester thus formed.

These cross linking agents may be written in accordance with the following formula:



in which X may be H, Cl or  $\text{CH}_3$  and Y may be H or  $\text{CH}_3$ . These variations in X produce respectively the acrylic, chloracrylic and methacrylic acid esters. If Y is H, the compounds are the vinyl acrylates and methacrylates, and if Y is  $\text{CH}_3$  this forms the isopropenyl acrylates and methacrylates. It will be appreciated that each of these compounds contains two of the unsaturated methylene groups  $\text{CH}_2=$  or the groups  $\text{CH}_2=\text{C}-$ .

The linear chain type of monomeric alkyl esters above defined may be copolymerized with the monomeric cross linking agent in desired proportions which preferably range from 0.5% to about 15% by volume of the cross linking agent, with the balance formed of the alkyl ester and with or without other polymerizable or non-polymerizable substances included therewith. A resin made wholly of the alkyl ester copolymerized with an appreciable amount of the cross linking agent tends to have a higher softening point or a greater degree of infusibility and less flow under heat and to present characteristics which are more suitable for grinding wheels than has the linear chain type of ester. The hardness on the Rockwell scale of methyl methacrylate varies from 55 to 57 and the addition thereto of 10% of vinyl methacrylate, for example, gives a hardness between 55 and 59; hence the variation in hardness is slight although the other properties as above discussed are materially improved.

These substances are preferably interpolymerized in such compatible amounts wherein the monomeric liquids are fully miscible and the polymerized product is a homogenous, substantially one-phase mass. For example, I may copolymerize from 1 to 15% by volume of vinyl methacrylate with methyl methacrylate, by heating the mixture with or without the addition of a polymerization catalyst, such as 0.02% of benzoyl peroxide, at a suitable temperature, such as 60° C. The product forms a transparent, colorless hard body which is well adapted for use as a grinding wheel bond.

As an example of one type of grinding wheel which may be made from such compounds, I may proceed as follows: A mixture is made of the desired proportions of methyl methacrylate and vinyl methacrylate and a slight amount of benzoyl peroxide as a catalyst. 490 grams of this

mixture is poured with 1656 grams of abrasive grains into an aluminum or stainless steel mold shaped to form a grinding wheel. The abrasive grains may be of any desired type, such as aluminum oxide or silicon carbide, and of any suitable grit size. The liquid quickly penetrates into the mass of abrasive grains, and wets them all but having a specific gravity less than the grains there will be a clear liquid above them. The mold is heated in an oven to 60° C. for a period of about 24 hours. The wheel may then be given a final bake at 110° C. for a period of 5 hours. Thereafter, the wheel is removed from the mold, bushed and trued as desired. The times and temperatures given are illustrative and may be varied widely with good results, those given being recommended.

For the manufacture of other types of grinding wheels I may produce first a solid interpolymer of the selected ingredients and mix the abrasive grains and the dry resin powder with a suitable plasticity developing medium, such as methacrylic acid, and shape a grinding wheel therefrom and thereafter complete the article by a suitable heat treatment. The bonding powder may be made as follows: To 33 c.c. of vinyl methacrylate and 570 c.c. of methyl methacrylate is added six-tenths of a gram of benzoyl peroxide. The mixture is then added to 1400 c.c. of carbon tetrachloride, in which it is completely miscible, and placed in a constant temperature bath maintained at 65° C. After an induction period of about five hours the copolymer, being insoluble in the carbon tetrachloride, begins to precipitate as a fine powder and is filtered off, washed with carbon tetrachloride and dried. I may also polymerize the mixture of vinyl methacrylate with methyl methacrylate to a massive piece and then crush and grind it to form a powder. I mix 1656 grams of abrasive grain with 500 grams of the above described powder and place in a mold. The mixture is pressed for thirty minutes in a hydraulic press with platens heated to 160° C. The wheel is then complete, the heat and pressure having softened and coalesced the resin, so that it forms with the abrasive grains an integral piece.

Other methods of procedure, such as set forth in the Kistler and Barnes application Serial No. 228,004 filed Sept. 1, 1938, of which I am one of the co-applicants, may be employed for producing suitable types of abrasive articles. For example, methyl methacrylate or other chosen linear chain type of alkyl ester and one of the cross linking agents may be mixed in desired proportions, such as 90 parts of the base substance and 10% of the cross linking agent, and this monomeric mass, together with 0.02% of benzoyl peroxide or other catalyst may be heated to 80° C. for about 1 hour. This viscous liquid is then mixed with the abrasive grains and the mass shaped as desired after which polymerization is completed. The plastic mass of abrasive grains and the partially polymerized bond may be shaped in a suitable mold and preferably with pressure required to give the desired structure. A shaped mass is thereafter heated, either within or outside of the mold, to complete the polymerization of the bond. This step may comprise heating the molded mass in an oven at 60° C., with or without the aid of light, for 24 hours to substantially complete the polymerization of the monomeric substance present; after which it may be given a further final

baking treatment at 100° C. or higher for a period of 5 hours or so. The temperature time conditions may be widely varied.

5 The porosity of the article depends upon the relative proportions of the abrasive grains and the bond, and the procedure set forth in the patent to Howe and Martin No. 1,983,032 may be adopted in order to make a controlled volume structure. The percentage by weight of 10 the bond in a grinding wheel may vary from 4 or 5% by weight for a very soft wheel to 30% or more for a harder wheel.

15 It will now be appreciated that the characteristics of the abrasive article will vary widely in accordance with the materials and proportions selected. For example, methyl methacrylate softens in the neighborhood of 100° C. depending upon the method employed for measuring the same and 10% of vinyl methacrylate interpolymerized therewith gives a softening point of 20 130° C. when similarly measured. The vinyl and isopropenyl acrylates provide somewhat softer bodies and have a lower softening point, but nevertheless these substances are useful as cross linking agents. For example, a bond of methyl 25 methacrylate used alone will smear over the face of a grinding wheel in a dry grinding operation. An interpolymer of that ester with 15% of vinyl acrylate, for example, softens at a lower point, but this interpolymer will not smear and thus is greatly superior in that characteristic. This results from the fact that an increase in the amount of vinyl or isopropenyl ester decreases the ability of the interpolymerized material to flow under heat. Hence, the interpolymer which is even softer than methyl methacrylate may be superior for certain types of 30 abrading operations.

35 It is also to be understood that I may utilize 40 other polymerizable substances in connection with the ones above discussed for the purpose of imparting other desired properties to the bond; and such other substances may be incorporated in the bond without departing from the 45 spirit and the scope of this invention; hence the claims are to be interpreted accordingly as not excluding the presence of such other substances. The above disclosure is therefore to be considered as illustrating the general principles of my 50 invention and preferred embodiments and compositions thereof and not as imposing limitations on the claims appended hereto.

55 This case is a continuation in part of my prior application Serial No. 227,108 filed Aug. 27, 1938.

I claim:

1. An abrasive article comprising abrasive grains united by a bond composed primarily of a resin formed of copolymerized substances comprising an ester of an alkyl alcohol having not over four carbon atoms per molecule and an acid selected from the group consisting of the acrylic, chloracrylic and methacrylic acids copolymerized with an ester selected from the group consisting of the vinyl and isopropenyl esters of one 60 of said acids.

65 2. An abrasive article comprising abrasive grains united by a bond composed primarily of a resin formed of copolymerized substances comprising an ester of an alkyl alcohol having not over four carbon atoms per molecule and an acid selected from the group consisting of the acrylic, chloracrylic and methacrylic acids copolymerized with a compatible and miscible 70 amount of an ester selected from the group con-

sisting of the vinyl and isopropenyl esters of one of said acids, said alkyl ester constituting the major portion of the mass and the bond being a substantially homogenous one phase substance.

3. An abrasive article comprising abrasive grains united by a bond composed primarily of a resin formed of copolymerized substances comprising an ester of an alkyl alcohol having not over four carbon atoms per molecule and an acid selected from the group consisting of the acrylic, chloracrylic and methacrylic acids copolymerized in the presence of the abrasive grains with from 0.5 to 15% of an ester selected from the group consisting of the vinyl and isopropenyl esters of one of said acids, said alkyl ester constituting the major portion of the mass and the bond being a substantially homogenous one phase substance.

4. An abrasive article comprising abrasive grains bonded as a porous integral body by a lesser amount of a bond composed primarily of a resin formed of copolymerized substances comprising an ester of an alkyl alcohol having not over four carbon atoms per molecule and an acid selected from the group consisting of the acrylic, chloracrylic and methacrylic acids copolymerized with not over 15% of a compatible and miscible amount of an ester selected from the group consisting of the vinyl and isopropenyl esters of one of said acids.

5. An abrasive article comprising abrasive grains bonded primarily by a resin formed of copolymerized substances comprising an ester of an acid selected from the group consisting of the acrylic, chloracrylic and methacrylic acids and an alkyl alcohol having not over four carbon atoms per molecule and branched as much as possible, which is interpolymerized with a lesser compatible and miscible amount of an ester selected from the group consisting of the vinyl and isopropenyl esters of one of said acids.

6. An abrasive article comprising abrasive grains bonded primarily by a resin formed of copolymerized substances comprising an ester of an acid selected from the group consisting of the acrylic, chloracrylic and methacrylic acids and an alkyl alcohol having not over four carbon atoms per molecule and less than a maximum branching which is interpolymerized with a lesser compatible and miscible amount of an ester selected from the group consisting of the vinyl and isopropenyl esters of one of said acids.

7. An abrasive article comprising abrasive grains bonded primarily by a resin formed of methyl methacrylate copolymerized with an ester selected from the group consisting of the vinyl and isopropenyl acrylates, chloracrylates and methacrylates.

8. An abrasive article comprising abrasive grains bonded primarily by a resin formed of methyl methacrylate copolymerized with from 0.5 to 15% by weight of vinyl methacrylate.

9. An abrasive article comprising abrasive grains bonded primarily by a resin formed of methyl methacrylate copolymerized with from 0.5 to 15% by weight of isopropenyl methacrylate.

10. An abrasive article comprising abrasive grains bonded primarily by a resin formed of methyl methacrylate copolymerized with from 0.5 to 15% by weight of vinyl acrylate.

CARL E. BARNES.